

Sept. 27, 1932.

C. E. BENNETT

1,879,867

LEAD PRESSING

Filed March 1, 1932



INVENTOR.

Charles E. Bennett,

BY

Kiddle Marston and Hornidge.

ATTORNEYS.

## UNITED STATES PATENT OFFICE

CHARLES E. BENNETT, OF HAWTHORNE, NEW JERSEY, ASSIGNOR TO THE OKONITE-CALLENDER CABLE COMPANY, INCORPORATED, OF PATERSON, NEW JERSEY, A CORPORATION OF NEW JERSEY

## LEAD PRESSING

Application filed March 1, 1932. Serial No. 595,990.

The present invention relates to an improvement in lead pressing apparatus and methods, and has for one of its objects the provision of a method as well as an apparatus whereby the working of lead and like materials is greatly improved.

In the sheathing of electric cables for instance, which is an intermittent operation, the cable is fed through the dies of the press as 10 the molten lead or other material is forced thereto, until the charge in the heating pot is exhausted, or nearly so. A small portion of the charge, however, is necessarily left in the pot and in the passage or passages leading 15 to the die. The press is stopped until a fresh charge of molten material is supplied to the reservoir or pot. During the interval between the stopping of the press and resumption of operations, that part of the charge 20 remaining in the press cools to a plastic or semi-solid condition and the upper surface of this "slug" becomes oxidized. The effect of this is that when a fresh charge of molten lead is placed in the pot an imperfect union 25 or weld is obtained, on resumption of operations, between the old charge or "slug" and the fresh charge. This imperfect weld or union is recognized in this art and various methods have been tried to overcome it. I 30 have determined to my own satisfaction that the reason for the imperfect union between the two charges is the presence of the oxides which form on the exposed surface of the old charge or "slug". With this in mind, therefore, I have provided a method whereby this 35 dross may be removed in a practicable manner, and I have actually produced welds or unions which cannot be seen under the microscope.

40 My improved method consists in melting the exposed surface of the "slug" and then flowing the next charge of molten lead or other material into the machine, the oxides and other impurities, which I shall term 45 "dross" and which float upon the molten surface of the slug simply rising or floating to the top of the fresh charge, so that I have pure lead to pure lead at the seam or union and hence will obtain a homogeneous perfect 50 bond or union. This melting of the exposed

oxidized surface of the "slug" of the preceding charge may be produced in a variety of ways. I have tried successfully an electric arc, an electric arc in a hydrogen flame and metal billets such as steel heated to a white 55 heat.

The drawing shows in part sectional elevation one embodiment of a suitable apparatus for the practice of my invention.

Referring to the drawing in detail, 1 designates the die blocks of a lead press, for instance, of usual construction. 2 is the pot or reservoir for the molten material. 3 is the usual fixed plunger for forcing the molten lead to the die blocks 1, the die blocks and 60 pot being raised, as usual, by hydraulic ram 4, the molten lead being forced to the die blocks under several tons pressure.

In the operation of such a machine the ram 4 is raised until the plunger or piston 3 forces 70 the bulk of the molten lead out of the pot 2. However, there is always a small amount of lead left in the pot, and of course the passageway from the pot to the die will be left 75 filled. This part of the charge is termed a "slug" in the lead press art.

After the first run of the press the pot and die blocks are lowered, and a new charge of molten lead dumped into the pot. In the meantime the slug 5 has cooled below a molten 80 temperature and may be considered in a plastic or semi-solid state, and in this cooling operation oxides and other materials accumulate or form on the upper exposed surface of the slug. Accordingly when a fresh 85 charge is dumped into the pot this dross prevents a good seam or weld between the leads of the two charges.

To overcome this imperfect bonding, I propose to melt the upper surface of the slug 5 90 before the next lot of molten lead is charged. In the drawing I have shown a billet for this purpose. This billet is heated to the necessary temperature, to white heat if desired, and then lowered into the pot 2, if necessary 95 into contact with the surface of the slug 5. In any event the surface of the slug to an appreciable depth is reduced to a molten condition and upon withdrawal of the billet while this surface is still in this condition a 100

fresh charge of lead is flowed into the pot, this fresh charge as it flows in displacing the dross on the molten surface of the slug the dross simply rising or floating to the top of [5] the fresh charge. Consequently I have pure lead to pure lead, and am assured of a perfect bond or union. As a matter of fact I have obtained such excellent results in practicing my invention, using a steel billet for melting 10 the surface of the slug, that the same is not visible under a microscope.

As above mentioned instead of the heating means shown, I may employ an electric arc, an arc in a hydrogen flame or other suitable 15 heating device or arrangement which will produce the desired melting of the surface of the slug.

What I claim is:—

1. In lead pressing the method which comprises applying pressure to a molten lead charge to force a portion of the same through 20 a die, relieving the pressure on the charge, then applying heat to the surface of the remainder of the charge until said surface be- 25 comes molten, and while the surface is in a molten state imposing a fresh charge of molten lead upon the same to displace the dross carried thereby, and then applying pressure to the fresh charge to form a homogeneous 30 bond or union between the two charges.

2. In combination an extruding press provided with an open reservoir for molten material, pressure means for forcing a portion of the molten charge out of the reservoir to 35 a die, and means for applying heat to the exposed surface of that portion of the charge remaining in the reservoir after the withdrawal of the said pressure means and before the introduction of a fresh charge of 40 molten material into the reservoir to reduce the said exposed surface to a molten condition, whereby introduction of the fresh molten charge will displace the dross carried on the said molten surface of the preceding 45 charge.

This specification signed this 27th day of February, 1932.

CHARLES E. BENNETT.